

May 20, 1924.

1,494,674

A. DWORZAK

CHEMICO-MECHANICAL PROCESS FOR MAKING AN UNALTERABLE WHITE PIGMENT

Filed May 26, 1919

FIRST FLOOR



SECOND FLOOR



THIRD FLOOR



INVENTOR ADOLPH DWORZAK,

by DR. George Orwig, ATTORNEY

Patented May 20, 1924.

1,494,674

# UNITED STATES PATENT OFFICE.

ADOLPH DWORZAK, OF ST. LOUIS, MISSOURI.

## CHEMICOMECHANICAL PROCESS FOR MAKING AN UNALTERABLE WHITE PIGMENT.

Application filed May 26, 1919. Serial No. 299,873.

To all whom it may concern:

Be it known that I, ADOLPH DWORZAK, a citizen of Russia, residing at the city of St. Louis and State of Missouri, have invented a new and useful Chemicomechanical Process for Making an Unalterable White Pigment, of which the following is a specification.

My invention relates to improvements in chemico-mechanical processes for making an unalterable white pigment and my object is to provide simple, economical and uniform chemical treatment therefor and to provide apparatus for uniformly and continuously 10 and uninterruptedly performing the several chemical steps, in a manner to continuously receive and convey raw materials through 15 the treatment steps to a continuous delivery of the finished product without manual 20 assistance.

For my process I take common zinc blende which I convert into a purified solution of zinc sulphate and I take common baryta rock which I convert into a purified solution 25 of barium sulphide and I then mix these two solutions at a proper temperature and in equimolecular proportion thereby producing 30 the double precipitate which forms my pigment. I then grind, wash and otherwise physically refine my precipitate thereby 35 making it suitable for its intended use.

In my drawing I illustrate, in plan, three 35 groups of mechanisms, which groups are by preference arranged one above another, as on the first, second and third floors of a building, so that I may economize in the 40 conveyance of substances from certain machines to subsequent machines, by gravity, and in my specification I employ numerals for designating the several mechanical treat- 45 ing means.

The zinc blende most suitable for my purpose is that containing about a sixty per cent (60%) metallic content. This I grind 45 on an ordinary differential roll indicated by the numeral 5, on the drawing, and which is fed with the zinc blende by an ordinary conveyor designated A, the differential roll being adjusted to deliver the mashed ore 50 of such fineness as to let it pass a 40 to 60 mesh screen. The pulverized ore is next conveyed by a chute B to a rotary roasting furnace 6 located by preference on the sec-

ond floor, it being fed to the furnace 6 by a continuous feeder 7 located at one end of 55 the furnace. The rotary furnace 6 is heated by fuel, which is fed from the opposite end through a fuel feeder 8.

As the ore enters the furnace 6 it is exposed to a graded system of temperatures 60 which at the entry end of the furnace is not to exceed 570° F. As it progresses through the furnace by means of a screw conveyor, up to about three fourths of the furnace length it meets increasing temperature until 65 at the three fourths point it is exposed to a temperature of about 1170° F. Thereafter the temperature within the furnace decreases toward the discharge end where the temperature is not to exceed 660° F. The 70 time during which the ore is treated is approximately six hours. The purpose of this roasting step in the process is to drive off the sulphur, bismuth, antimony and any other volatile impurities. 75

The thus roasted and oxidized ore is gravity delivered from the furnace 6, and at the delivery temperature, to an enameled trough 9.

At this point dilute sulphuric acid is 80 added for the next step in my process. In order to make an acid solution of the proper strength I provide a lead lined tank 10 with an agitator 11 which tank has a delivery pipe 12 controlled by a valve 13. In this tank 85 I prepare a mixture of sulphuric acid and water, the condensate from certain or various of the heating coils employed in my process, to a specific density of 1.160. The trough 9 is equipped with a screw conveyor 90 so arranged as to move the roasted ore for its delivery from the trough 9 and at the same time thoroughly mix it with the acid solution. The trough 9 is provided with exterior heating coils which maintain the mixture of roasted ore and sulphuric acid at a 95 temperature of about 300° F.

The screw conveyor also is heavily enameled to protect it from the corrosive action of the sulphuric acid. 100

From trough 9 by means of its screw conveyor the mixture of ore and acid is delivered to a series of oblong, closed topped treatment tanks designated by numerals 14, 16 and 18. Each tank 14, 16 and 18 is provided with a screw conveyor designated 15, 105

17 and 19 and both the interior of the tanks as well as all exposed parts of the screw conveyors are protected from corrosive action of the acid either by lead covering or by 5 heavy enameling.

When the mixture of roasted ore and sulphuric acid is delivered to the tank 14 there is a certain amount of sedimentation and in order to conveniently handle both 10 the sediment and supernatant liquor I make these tanks of a novel shape namely that of a truncated substantially square, pyramid which I place with its major axis at an angle of approximately ten and three fourths degrees to the horizontal.

The action of the screw conveyor is that of moving the sediment upwards on the given degree toward the end of the truncated pyramidal tank from which it is ejected into 20 the larger end of an exactly similar tank 16 with its conveyor 17. At this point I add fresh dilute sulphuric acid from tank 10. The delivery from tank 16 is to tank 18 in which an exactly similar step is conducted, 25 but in which tank the last metallic zinc out of the treated (roasted) zinc ore, is separated by its treating solution, namely the dilute sulphuric acid.

The conveyor 19 of tank 18 delivers the 30 treated ore to a sump pit 20 where it is washed to recover any zinc left, with water, the condensate previously referred to, and the wash water removed by a pump 21 to tank 14.

35 During the step of treatment in the tanks 14, 16 and 18 the dilute sulphuric acid converts the zinc content of the roasted ore into soluble zinc sulphate which is carried along in solution. In order that this effect 40 may obtain it is necessary that the content of these treatment tanks shall be heated to boiling point and to this end the tanks are provided with lead coils fed with steam.

The liquor containing the zinc as sulphate 45 is pumped from the third of the series of tanks 18 by a pump 22 to tank 23. In tank 23 the zinc liquor is diluted with water (of condensation) and agitated until it is of a specific density of 1.380. The sulphuric acid treatment as above recited yields a solution of the zinc blende and according to the proportion of ore and acid this solution may or may not contain free acid. Free acid is 50 objectionable to my process and if it be found here it is at this point to be neutralized by the addition of more zinc blende until a neutral solution is produced which neutral solution I call my zinc liquor.

55 By the above recited series of steps I have 60 extracted from the zinc blende all of the available zinc and have adjusted the specific density of its solution to a point best adapted to my process of making unalterable white pigment and the sludge is drawn off at the bottom of said tank to pit 20 from which it

may be discarded or returned to be retreated if its zinc content justifies.

The zinc liquor as thus prepared contains extraneous and objectionable compounds, which as is well known to those versed in 70 the art, cause by their chemical changes, reactions, or deteriorations, a degradation from pure white and it is therefore essential to the process of making an unalterable white that these be eliminated. The zinc 75 liquor in tank 23 is therefore conducted from the top of the tank to an enameled or lead lined tank 24.

An intermediate step at this point is an electrolytic one, which takes place in the 80 electrolytic cells 23a. The purpose of the electrolysis is that of the elimination of copper, and other bases of corresponding electrolytic potential. Bases of the copper potential class are first electrolytically deposited at relatively low voltages, while such bases as cadmium may similarly be electrolytically deposited but, with increased voltage, the application of heat and as an adjunct agitation by heated air, all in the 85 presence of powdered zinc which is then added in the tank 24 in which there occurs a second electrolytic treatment.

The zinc liquor now freed from the above 90 mentioned bases and held in tank 24 is boiled by lead coils fed with steam and agitated by an air agitator which may be fed with hot air, or, should it be desirable to lower the temperature quickly, with cold air.

Much of the impurities that have been 100 thrown down by electrolysis and the zinc dust are held in suspension in the zinc liquor wherefore it becomes necessary to remove them. The zinc liquor is therefore pumped from the tank 24 by a pump 27 to a filter 105 28, where the several impurities mentioned above are removed from the zinc liquor.

The step of boiling in the tank 24 by heat- 110 ed coils 25 and agitation by air agitator 26 and pumping by pump 27 and filtering by 115 filters 28 is twice repeated by duplicate apparatus, including tank 30, with its heating coil and agitator, pump 31, filter 32, and tank 33 with its heating coil and agitator, pump 34 and filter 35.

In tank 30 barium carbonate is added in sufficient quantity to react with, and precipitate any iron that may be present and electrolysis is applied to precipitate any other impurities which may settle out through the former action. In tank 33 there is made an addition of red lead for the purpose of reacting with and precipitating manganese. Thus it will be seen that after treating the zinc blende to make a zinc liquor which liquor contains objectionable impurities I remove these impurities by three independent chemico-electrolytic actions.

These said actions differ from one an- 130

other in their impressed voltages, each voltage being appropriate to its particular electrolytic step and which actions are performed in the presence of an additional appropriate reagent.

5 The resulting liquor is then cooled with air and tested for neutrality and if found acid the acid condition is neutralized by the addition of zinc oxide and the foregoing 10 neutralizing step is adjusted to give a neutral solution at this step.

The liquor is now diluted with water (the condensate) to adjust its specific density to 1.283.

15 The liquor thus prepared consists primarily of zinc sulphate solution after passing through the filtration step 35 and is now suitable for the preparation of my unalterable white pigment and is stored in 20 tank 36 for use later in the process.

Concurrent with the preparation of the above described zinc sulphate solution I 25 prepare a barium sulphide solution. This solution is prepared by taking crude baryta rock, pulverizing it in an ordinary pulverizer 37, to a fineness corresponding to 100 mesh screen. Coal is likewise pulverized, the grade of coal being such as to contain not less than 14000 B. t. u. per pound.

30 The baryta rock and the powdered coal are thoroughly mixed in a mixer 38. The proportion of ground baryta rock and ground coal is approximately 70 per cent of the former and 30 per cent of the latter 35 which proportionality depends upon the barium content of the baryta and the sulphur content of the coal. This mixed powder is wetted with just sufficient water to form a paste and this paste is gravity fed 40 to a long rotary furnace 39 through which it travels continuously, this furnace is in all respects similar to furnace 6, used in the treatment of the zinc blende, but in the treatment of the baryta and coal mixture 45 the maximum temperature is approximately 1600° F. and exposed for a much shorter period, namely two and one half hours.

By this step, the baryta rock is converted 50 into barium sulphide which is soluble. The material thus treated is delivered from the furnace 39 to a heated trough 40. The whole step herein recited being identical with the parallel step in the described zinc treatment.

55 From the trough the baryta product is delivered to a series of three truncated, square, pyramidal lixiviators similar in all respects to tanks 14, 16 and 18 and their screw conveyors 15, 17 and 19, where the barium sulphide is extracted, the menstruum being water.

60 After the completion of this extraction in the series of lixiviators, the liquor is pumped by pump 41 through filter 42 which 65 filter separates the barium sulphide held in

solution from any sludge generated by the ash content of the coal, which sludge may have been carried along with the barium sulphide solution. In order to free the barium sulphide from most of the sludge 70 it is passed through a tank, in all respects similar to the tank 20, from which tank the pump 41 is fed.

The barium sulphide liquor thus freed from foreign insoluble matter is finally 75 stored in tank 43 and this solution forms the companion solution for the zinc sulphate solution stored in tank 36. In order that this solution may chemically fit the adjusted zinc sulphate solution it is diluted 80 with water (the condensate) to a specific density of 1.151. This barium sulphide liquor being near the point of saturation and consequent crystallization must be maintained at a temperature of at least 125° F. 85

As has been previously stated this process consists in an equimolecular precipitation between zinc sulphate solution of a specific density, by preference 1.283 and a barium sulphide solution of specific density of, by 90 preference, 1.151 and it may be determined by simple chemical considerations that equimolecular balance is established when such solutions are mixed in the proportion of 1109 parts of the one to 1891 parts of the 95 other, respectively.

In order to insure complete solubility of these reagents and to insure most favorable chemical action between them I effect this 100 reaction at the boiling point of the solutions and in order to further simplify my process I use the tanks 36 and 43 as measuring tanks and they are therefore of sizes corresponding to the proportionality above recited.

In effecting the mixture of these two solutions I first admit the proper amount of zinc sulphate into the mixing tank 45 and immediately thereafter I admit the barium sulphide solution to the same tank. It being desirable to admit the barium sulphide solution quickly the tank 43 is therefore provided with an adequately large delivery pipe. I provide tank 45 with an agitator 46 to insure very active agitation and in 110 order to insure a complete double precipitation I continue to agitate the mixture for no less than 15 minutes. The zinc sulfate and the barium sulfid react upon each other in the well-known manner to form a precipitate of zinc sulfid and barium sulfate.

At the completion of this reaction I pump the mother liquid and its precipitate, by pumps 49 and 50, to a battery of filters 51, 52, 53 and 54. The filtrate being conserved in an appropriate tank and the precipitate being conveyed to rotary dryer 57. My product is now in its highest state of purity for which reason the interior of dryer 57 is enameled. This dryer is heated, either 125 130

by waste gases from earlier steps in the process, or by steam, and maintained at a temperature of approximately 300° F.

Connected with dryer 57 is a suction fan 58 whose purpose is to remove the water vapor generated in the drying. In order that the drying process may be continuous the interior of the dryer is provided with a helical flight whereby the material in the act of drying is moved longitudinally of the dryer and toward its discharge end. By this specific arrangement I avoid a continuous mixing of the thoroughly dried precipitate with moist precipitate.

15 The precipitate, when thoroughly dried dumps out of the discharge end of the dryer directly into the bin 59 and the communication between the dryer 57 and bin 59 is so constructed that this last operation is out 20 of contact with the atmosphere. Communicating with the bin 59 at the bottom there is a drum provided with only one opening which opening shall not exceed in dimension one fifth of the drum circumference. This 25 drum fits accurately as may be the bottom of the bin and is air sealed to it against atmosphere. When the drum has been filled with precipitate it is revolved so that the opening descends to a lowermost position 30 discharging the precipitate into a second bin whereupon it is returned to its former position to receive a new charge.

Contained within the last mentioned bin 35 is a pair of ribbed rolls through which the precipitate in its course of travel must pass. The purpose of these rolls is to crush the precipitate so that no particles of it shall be larger than  $\frac{1}{8}$  of an inch.

After the crushing, the precipitate is delivered by gravity and out of contact with air to kiln 60 which is revoluble where the crushed precipitate is reheated for calcination to a temperature of 1000° F. for a period of thirty minutes and any residual moisture is driven off, extracted and removed by exhaust fan 58 (which keeps a certain vacuum in the furnace), all out of contact with the atmosphere. The exhaust fan produces a partial vacuum in the kiln 60, so that calcination proceeds under a partial vacuum. After the precipitate has been finally dried and highly heated it is dumped from exit end 61 of kiln 60 into cold water tank 62. The cold water quenching tank is so disposed that any steam generated by quenching the highly heated precipitate may not enter the kiln 60 and also prevents contact with air.

In this last kiln (60) roasting any possible sulphur content in the precipitate is driven off and should there be any other substances aside from the highly refractory double precipitate this process of calcination volatilizes them.

65 When the pigment falls into the cold wa-

ter of the tank 62, should there remain any refractory soluble matter it will be dissolved, and to secure the thorough elimination of any such soluble matter as well as to insure rapid cooling this water is constantly renewed. The tank 62 and the remaining tanks 63 and 64 of this series are in all respects similar to the truncated, square pyramidal tanks 14, 16 and 18, and the pigment served to these tanks is handled in a corresponding manner and finally delivered to a sump pit 65.

From the sump pit it is pumped by pump 66 to a battery of wet grinding mills 67 where it is ground to a fineness corresponding to 200 mesh. From the delivery of the battery of the mills 67 the pigment passes on to a rotary screen 68 where a constant stream of water is played on the ground pigment, returning the coarse material to 85 pit 65 whence it is again pumped to mill 67 to be reground.

The material of requisite fineness which passes through the screen 68 falls into a tank 69 and thence to a series of tanks 70, 80 similar to the tanks 14, 16 and 18. From this system of tanks 70 the liquid containing the pigment runs into concrete pits 71 where the pigment is washed permitting the elimination of any alkaline salts or other 85 foreign matter. The washing in tanks 71 is by means of water which is constantly fed in from the bottom and this washing is assisted by air agitation.

This water bearing any soluble impurities 100 flows away over the tops of the tanks.

The washing is continued till the water shows no chemical reaction. The pigment is then collected in pit 72 from which it is removed by pump 73 through pipe 74 to 105 tank 75, which tank is of large diameter and provided with a hopper bottom, this hopper bottom is provided with pipe 76 and a valve connected to pump 77 which delivers the pigment to the filter 78. The purpose 110 of the tank 75 is to permit the sedimentation of the pigment so that the pump 77 and the filter 78 may handle a minimum of liquid. The pigment which is caught in filter 78 is conveyed by a pipe 80 from which 115 the pigment is pressed into a dryer 81, similar to the dryer 57.

From the dryer 81 the pigment is gravity fed to pulverizing mills 82 which again pulverize the material to a fineness of a 200 120 mesh screen.

The reground pigment is delivered to a bin 83 either by a conveyor or blower fan 84, and the now finished pigment is ready for packing.

I claim—

1. The process which consists in causing to react upon each other at substantially their boiling temperature, a pure aqueous solution of zinc sulfate and a pure aqueous 1

solution of barium sulfid, separating the resulting precipitate from the liquid, and drying the separated precipitate.

2. The process which consists in causing a pure aqueous solution of zinc sulfate to react upon a pure aqueous solution of barium sulfid, separating the resulting precipitate from the liquid, drying such separated precipitate, crushing it, and then subjecting it to calcination at a temperature higher than that used during the above-mentioned drying operation.

3. The process which consists in causing solutions of zinc sulfate and of barium sulfid to react upon each other, separating the resulting precipitate from the liquid, drying such separated precipitate, crushing the dried product and then subjecting it to a temperature higher than that used during the above-mentioned drying operation, quenching the hot product, grinding and washing the quenched product, separating the liquid from the solids, and finally drying and grinding such solids.

25 4. The process which consists in causing to react upon each other, a pure aqueous solution of zinc sulfate of a density of 1.283,

and a pure aqueous solution of barium sulfid of a density of 1.151, separating the resulting precipitate from the liquid, and drying the separated precipitate. 30

5. The process which consists in causing to react upon each other at substantially their boiling temperature, a pure aqueous solution of zinc sulfate of a density of 1.283 35 and a pure aqueous solution of barium sulfid of a density of 1.151, separating the resulting precipitate from the liquid, drying the precipitate at about 300° F., crushing the dried precipitate and then heating it for 40 calcination, to about 1000° F. under exclusion of air, quenching the hot calcined product in cold liquid, grinding and washing the quenched product, separating the liquid from the solids, and finally drying and 45 grinding such solids.

6. The process which consists in causing to react upon each other, solutions of zinc sulfate and of barium sulfid, separating the resulting precipitate from the liquid, drying the precipitate, crushing the dried precipitate, and then calcining it under a partial vacuum. 50

ADOLPH DWORZAK.